

# United States Patent [19]

Micheletti

[11] 3,775,269

[45] Nov. 27, 1973

[54] SELF-COLORING ANODIC OXIDIZING  
PROCESS FOR ALUMINUM AND FOR  
ALLOYS THEREOF

[75] Inventor: Ciro Micheletti, Novara, Italy

[73] Assignee: Societa' Per L'Esercizio Dell'Istituto  
Sperimentale Metalli Leggeri, Milan,  
Italy

[22] Filed: Mar. 14, 1972

[21] Appl. No.: 234,683

[30] Foreign Application Priority Data  
Mar. 15, 1971 Italy ..... 21754 A/71

[52] U.S. Cl. ..... 204/58

[51] Int. Cl. ..... C23b 9/02

[58] Field of Search..... 204/58, 262, 274

## [56] References Cited

### UNITED STATES PATENTS

3,634,213 1/1972 Coates ..... 204/58

3,616,311 10/1971 Barkman et al. ..... 204/58

## OTHER PUBLICATIONS

The Surface Treatment and Finishing of Aluminum by  
Wernick et al. 1964, page 314. al.,

Primary Examiner—John H. Mack

Assistant Examiner—R. L. Andrews

Attorney—Richard K. Stevens et al.

## [57] ABSTRACT

An improved self-coloring anodic oxidation process  
for aluminum and its alloys utilizing an electrolytic  
bath in which the electrolytic cell is subdivided by a  
porous baffle into an anodic and a cathodic compart-  
ment, the improvement comprising maintaining the  
electrolytic solution in the cathodic compartment at a  
temperature lower than that of the anodic compart-  
ment.

1 Claim, No Drawings

**SELF-COLORING ANODIC OXIDIZING PROCESS  
FOR ALUMINUM AND FOR ALLOYS THEREOF**

The present invention relates to an improvement in self-coloring anodic oxidizing process for aluminum and its alloys, an improvement that reduces the consumption of the components of the electrolytic system used and substantially eliminates precipitate formation from said system.

It is known that aluminum and its alloys may be 10 coated with layers of oxide of considerable thickness and high resistance, by an electrolytic treatment in aqueous solutions in which the aluminum acts as an anode.

Moreover, it is also known that by using as electrolytes solutions based on carboxylic acids of the aliphatic series, it is possible to obtain self-colored layers by transformation and incorporation in said layers of the constituents and alloying elements present in the material to be oxidized.

The self-coloring anodic oxidizing processes so far suggested, amongst which may be particularly mentioned, are the MS-process, based on a binary mixture of maleic acid and sulfuric acid, the MOS-process based on a ternary mixture formed of maleic acid, oxalic acid and sulfuric acid, as described in Italian Patent No. 793,929, and in Belgian Patent No. 660,867, and the TOS-process based on a ternary mixture of tartaric acid, oxalic acid and sulfuric acid, as described in Italian Patent No. 720,028, have all in common a serious drawback, that is, to give rise during the course of the oxidation, to cathodic and/or anodic decomposition by-products of the aliphatic carboxylic acids used, with the consequence of heavy consumptions of the components thereby affected, of an increase in processing costs, and appreciable variations in the reproducibility of the coloration.

Said decomposition reactions lead in some instances to the complete fission of the carboxylic acid or to its transformation to soluble products (such as is the case with oxalic acid in the TOS and MOS-processes). In other cases, on the contrary, there takes place a conversion of the affected carboxylic acid into difficultly soluble products (such as is the case with maleic acid in the MOS- and MS-processes), with the consequent formation of precipitates in various parts of the installation and consequent clogging (particularly of the perforated pipes used for the compressed air stirring of the electrolyte) and a lowering of the exchange capacity of the refrigerating apparatus and of the resin columns used for eliminating the aluminum from the baths.

In order to reduce the drawbacks indicated above, it has already been suggested by the applicant, in Italian Patent No. 846,035, an improvement consisting of placing in the electrolytic cell, used for carrying out the anodic oxidation process, a porous baffle immersed into the electrolytic solution used in the process, said porous baffle subdividing the electrolytic cell into two compartments, an anodic one and a cathodic one. By this expedient there is achieved a reduction of 40 percent in the consumption of the maleic acid in an electrolytic bath based on maleic and sulfuric acid.

By using the above-mentioned porous baffle, there still remains, even if reduced, the formation of precipitates in the cathodic compartment.

An object of this invention is that of providing an improvement in a self-coloring anodic oxidizing process

for aluminum and its alloys, by which improvement the above-mentioned drawbacks are reduced.

More particularly, an object of this invention is that of providing a process that will reduce to a minimum the formation of precipitates from the electrolytic solution and consequently reduce harmful clogging phenomena in the installation and the reduction of the exchange capacity of the refrigerating apparatus and of the ion-exchanging resin columns.

Still another object of this invention is that of reducing the consumption of the components of the electrolytic system used, also obtaining thereby an improved uniformity of the composition of the electrolytic system and, thus, a better reproducibility of the colorings obtained in the anodic coating, without having to resort to frequent and expensive additions to the electrolyte.

These and still other objects of the invention will become still more apparent to those skilled in the art from the following detailed description, and are conveniently achieved through the present invention wherein the electrolytic cell is subdivided by a porous baffle into two compartments, an anodic one and a cathodic one, and wherein according to the improvement of this invention the electrolytic solution of the cathodic compartment is maintained at a temperature that is lower than that of the anodic compartment.

During the tests carried out in order to examine the cathodic and anodic reaction mechanisms of the di- and tri-acid baths affected by the decomposition of the components thereof, it was, in fact, surprisingly found that if the temperature of the catholyte is maintained below the working temperature of the anolyte, there occurs a heavy decrease in the decomposition kinetics of the electrolyte components subject to such a phenomenon, and, thus, there occurs a substantial drop in the consumption of the bath components affected by these decomposition reactions.

During said tests there was also observed a considerable reduction of precipitates in the cathodic compartment.

The electrolytic solution used in the cell includes a carboxylic acid which may be selected from among the following acids: maleic, oxalic, tartaric acid, either alone or in a binary or ternary combination, and generally in the presence of sulfuric acid.

The porous baffle that subdivides the cell into two compartments, a cathodic one and an anodic one, as already described in Italian Patent No. 846,035 by the same applicant, is of a material resistant to the corrosive action of the electrolytic system used, preferably being composed of polyethylene, glass or a ceramic material. Said baffle has pores having a diameter comprised between 0.1 and 50 $\mu$ .

The difference of temperature or thermal gradient between the electrolytic solutions of the two compartments, the anodic one and the cathodic one, is in general achieved by cooling down the cathodic compartment with respect to the anodic one.

Said cooling down may be achieved by circulating a liquid coolant inside a sleeve surrounding the cathodic compartment, or in a coil immersed in the cathodic compartment, or by means of any other equivalent suitable means.

In case a coil immersed in the cathodic compartment is used, said coil, like the porous baffle, will have to be made of a material resisting the corrosive action of the electrolytic system used. Preferably, it is made of the

same material of which the cathode is made, e.g., of stainless steel, graphite or aluminum.

Moreover, the refrigerating system and the cathode may form one single element of the cell, the cooling coil being incorporated into the cathode itself.

It has been found that, to obtain the best results, the temperature of the electrolytic solution in the cathodic compartment must be kept below 22° C.; such a temperature must be, however, higher than the temperature causing freezing of the electrolytic solution used in the cell.

During tests carried out, it was found that the use of the porous baffles combined with the cooling of the cathodic cell, especially in the case of the MS and MOS processes, offered considerable advantages without, however, involving on the other hand too heavy building and maintenance costs. The advantages of the present invention may be thus concisely summarized:

1. Elimination of precipitates, in the case of the MS and MOS processes, in the anodic zone, and all the drawbacks derived from such precipitates;

2. Considerable reduction, still in the case of the MS and MOS processes, of the precipitates also in the cathodic zone;

3. A reduction of consumption (in all mentioned processes) of the components affected by the secondary reactions of the electrolytes;

4. A reduction in ancillary equipment and in their maintenance in connection with the precipitates.

For an even clearer illustration of the present invention and the advantages therefrom derived, the following example of an embodiment of the invention will now be given.

#### EXAMPLE

The anodic oxidation was carried out at 1.5 A/dm<sup>2</sup>, at 20° C. and for 45 minutes, in a self-coloring bath of the MS type consisting of an aqueous solution and maleic and sulfuric acid of the following composition:

maleic acid: 300 g/l

sulfuric acid: 3 g/l

The cell was subdivided by a porous polyethylene baffle having pore-diameters comprised between 7 and 10 $\mu$ . In the cathodic compartment was arranged 6 cathodes consisting of AISI 316 stainless steel pipes of such a surface as to ensure that the cathodic current density be of at least 1.5 A/dm<sup>2</sup>.

Through these pipes forming the cathodes was made to circulate a refrigerating liquid so as to maintain the temperature of the electrolytic solution of the cathodic compartment constantly at 17° C.

In the self-coloring bath were oxidized various samples until attaining an aging of the bath of about 70 Ah/l.

After this aging, it was observed that in the anodic compartment no formation of precipitates had taken

place and that in the cathodic compartment the formation of precipitates was considerably reduced.

Moreover, it was also found that the consumption of maleic acid was lower by about 60 percent in comparison with that found in a similar bath without the porous baffle and the cooling of the cathodes and by about 20 percent in comparison with that found in a similar bath with the porous baffle but without the cooling of the cathodes.

In the following Table 1 the results of a series of tests are reported; these tests were carried out in a similar manner to the preceding Example and using different thermal conditions. For said tests a porous baffle having pore-diameters of 35-45 $\mu$  was used. The consumption of maleic acid as well as the formation of precipitate generating substances reported in the table are the values obtained after bringing the bath up to its operating conditions.

TABLE 1

| Test No. | Temperature of the anodic compartment (° C.) | Temperature of the cathodic compartment (° C.) | Consumption of maleic acid (g./Ah) | Formation of precipitate generating substances (g./Ah) |
|----------|----------------------------------------------|------------------------------------------------|------------------------------------|--------------------------------------------------------|
| 1.....   | 22                                           | 22                                             | 1.5-2                              | 1 ca. 0.8                                              |
| 2.....   | 22                                           | 20.5                                           | ca. 1                              | 1 ca. 0.1                                              |
| 3.....   | 28                                           | 20.5                                           | ca. 1                              | 1 ca. 0.1                                              |
| 4.....   | 35                                           | 20.5                                           | ca. 1                              | 1 ca. 0.1                                              |
| 5.....   | 30                                           | 18.5                                           | ca. 1                              | 1 ca. 0.1                                              |
| 6.....   | 22                                           | 17                                             | ca. 1                              | 1 ca. 0.1                                              |
| 7.....   | 20                                           | 17                                             | ca. 1                              | 1 ca. 0.1                                              |
| 8.....   | 22                                           | 14                                             | ca. 1                              | 1 ca. 0.1                                              |
| 9.....   | 22                                           | 4                                              | ca. 1                              | 1 ca. 0.1                                              |
| 10.....  | 22                                           | -4                                             | ca. 1                              | 1 ca. 0.1                                              |
| 11.....  | 35                                           | 22                                             | 1.5-2                              | 1 ca. 0.8                                              |
| 12.....  | 25                                           | 23                                             | 1.5-2                              | 1 ca. 0.8                                              |
| 13.....  | 35                                           | 23                                             | 1.5-2                              | 1 ca. 0.8                                              |

<sup>1</sup> Only in the cathodic compartment.

35 It will be understood that it is intended to cover all changes and modifications of the example of the invention herein chosen for the purpose of illustration which does not constitute departures from the spirit and scope of the invention.

40 What is claimed is:

1. In the process for self-coloring anodic oxidation of aluminum and its alloys by means of an electrolytic bath consisting of an aqueous solution of maleic and sulfuric acid, the improvement comprising

45 placing a porous baffle immersed in the electrolytic solution used into the electrolytic cell, said baffle having pores of a diameter between 0.1 and 50 $\mu$  and subdividing the cell into an anodic and a cathodic compartment;

maintaining the electrolytic solution in the cathodic compartment at a temperature below 22° C. and lower than that of the anodic compartment but higher than the temperature causing the freezing of the electrolytic solution used in the cell; and

55 applying direct current between the workpiece as the anode and the cathode.

\* \* \* \* \*